

## UNITED STATES PATENT OFFICE

2,202,531

## COATING STEEL

Vincent T. Malcolm, Indian Orchard, Mass., assignor to The Chapman Valve Manufacturing Co., Indian Orchard, Mass., a corporation of Massachusetts

No Drawing. Application July 12, 1939,  
Serial No. 284,091

2 Claims. (Cl. 148—6.5)

This invention relates to improvements in steels and is directed more particularly in methods of treating or coating steels to provide a protective coating therefor.

5 The principal objects of the invention pertain to a method of treating steels such as ordinary austenitic carbon and alloy steels in such a way as to provide a protective coating having characteristics rendering the same generally 10 resistant to corrosion.

According to the invention in its broad aspects the steel to be treated or coated is immersed in a solution having novel characteristics and subjected to heating temperatures for a length of 15 time.

The solution according to the invention includes electrolytic sodium hydroxide, sulphur and phosphoric acid, previous to which the steel is cleaned or degreased.

20 As an example the steel may be cleaned or degreased in carbon tetrachloride. Other cleaning substances or compounds may be used but in order to obtain the desired results the cleaning must be reasonably thorough.

25 The solution according to the invention may be as follows:

|                               | Grams |
|-------------------------------|-------|
| Electrolytic sodium hydroxide | 100   |
| Water                         | 100   |
| 30 Powdered sulphur           | 1     |
| Phosphoric acid               | 5     |

The solution which may be called a coating solution is preferably prepared by dissolving the 35 sodium hydroxide in water and then adding the sulphur and phosphoric acid to the same. The solution is preferably heated for at least one hour at a temperature of at least 250° F.

The steel to be coated is immersed in the coating 40 solution for a time depending on the size or area thereof to be coated. Steel pieces or work of different sizes or shapes will require different times of treatment and different temperatures may be used.

As one example of what has been done, a piece of steel 2" long, 1" wide and  $\frac{1}{4}$ " thick was soaked in the coating solution for approximately one-half hour with the temperature of the solution in the neighborhood of 270° F.

5 The result was a coating which was substantially black and which impregnated the surface of the steel to a marked extent. The coating taken on by the steel had a thickness of from .001" to .003" and had very desirable corrosion-resistant qualities in respect to mineral and organic acids as well as the basic solutions.

As instances the coating was resistant to the standard solutions of 4% sodium chloride, magnesium chloride, and salt spray solutions when 15 exposed for a 72 hour period to a spray thereof.

The color of the coating is very pleasing and not at all objectionable. It is readily and easily applied without the necessity for expensive equipment or materials so that the cost of coating is 20 very low.

Having thus described my invention, and the best manner of practicing the new process of forming this novel composition, but without limiting myself to the order of steps of such process 25 recited, or to the proportions of parts employed therein, or to the precise ingredients named, as it is evident that each of these ingredients has a considerable range of equivalents and that the order and proportions of the process may be 30 varied without departing from its scope and purposes.

I claim:

1. A bath for treating steel to provide a substantially black-colored protective coating thereon made from substantial amounts of sodium hydroxide and water and relatively small amounts of sulphur and phosphoric acid.

2. A bath for treating steel to provide a substantially black-colored protective coating thereon made from about 100 grams each of water and sodium hydroxide and about 1 gram of sulphur and about 5 grams of phosphoric acid.

VINCENT T. MALCOLM.